

## UNITED STATES PATENT OFFICE

2,422,038

## ANODES FOR INTENSIVE ARCS

Jean Francois Parisot, Paris, France, assignor to  
 Societe: Le Carbone Lorraine, a corporation of  
 France

No Drawing. Application July 25, 1945, Serial No.  
 607,093. In France January 17, 1942

15 Claims. (Cl. 176—121)

1

In a number of prior French Patents of "Le Carbone Lorraine" anodes for intensive arcs are described which are constituted by a tubular casing termed the bark or sheath which is made of commercially pure carbon and of a central core formed by a special composition contained inside said sheath.

These anodes, when submitted to an electric arc producing a current density of about 0.6 to 1.2 amperes per square millimeter of their cross sectional area, may produce spontaneously the phenomenon generally termed "Beck effect." It is known that this phenomenon appears when the density of current is gradually increased; it is characterized by an elevation of a few volts in the voltage drop in the arc, by a deepening of the crater reaching about one half of the diameter of the anode, by a considerable brilliancy of the gaseous mass at the bottom of the crater, by a rapid increase of this brilliancy when the density of current increases and finally by a particular appearance of the anodic flame.

In the French Patent 770,345 of June 9, 1933, Le Carbone Lorraine has described an anode the core of which is formed by a body of carbon to which is incorporated silicon or silicon carbide. The same applicant company has described in the French Patent 797,208 of January 25, 1935, a core containing one or more metals the atomic number of which is comprised between 22 and 29 and eventually compounds of rare earths.

The comparison of the intensive arc anodes established in conformity with the above mentioned patents, with normal intensive arc anodes the core of which is mineralized with fluorides or oxides of rare earths, has shown that silicon or silicon carbide reduces by about 40 to 60% the brilliancy produced by the standard anodes, whereas metallic iron causes only a 10 to 20% loss of this brilliancy. On the contrary, it is possible to rise by 5 to 20% above the standard anode brilliancy by associating in suitable proportions the iron and rare earths in the core.

Experience has shown however that the anodes having a core containing metallic iron show certain drawbacks. Pulverulent iron is oxidized either before or after its incorporation in the anode. During operation, this iron oxide is reduced in the vicinity of the crater, and sparks of molten metal spurt out and are blown away by the reduction gases so that metal particles may engage the optic system of the projecting apparatuses and become incrusted therein.

My invention has for its objects to remove this drawback and to further the manufacture of the

2

anode. It consists in principle in replacing the iron by certain nonoxydable ferrous alloys containing in particular one or more metals the atomic numbers are comprised inclusively between 22 and 28.

Such are chromium and nickel-containing austenitic or martensitic steel containing eventually other metals such as aluminium, together with carbon, silicon, etc.

However, these stainless alloys are tough and difficult to crush; on the other hand the presence of important contents of nickel and chromium increases to an exaggerated degree the green radiations in the light.

In conformity with my invention, I may replace iron by nonoxydable ferrosilicon which it is easy to crush. I have just stated that silicon considerably reduces the luminous efficiency of the intense arc in contradistinction with iron.

It was therefore not possible to foresee that the application to the anodes of ferrosilicon rich in silicon might lead to an advantageous luminous efficiency as disclosed hereinafter. Experience shows that from this standpoint, ferrosilicon acts substantially in the same manner as iron even with a proportion of 2 atoms of silicon for 1 atom of iron, in spite of the higher proportion of silicon.

Commercial ferrosilicons belong generally to the types 20-25%, 40-50% or 70-80% of silicon. All are inoxidable and unaltered in the presence of moist air and they resist the chemical attack of most acids. They are crushed to an increasingly easy degree when their contents in silicon increases. The intermediary type containing 40-50% of silicon corresponds substantially to the formula: Si<sub>2</sub>Fe.

The manufacture of my improved intensive anodes may be executed in accordance with the known methods.

The carbon sheaths are first prepared and a thick paste is injected therein which is constituted by subdivided carbon, pulverulent ferrosilicon and an organic binder. This paste may include moreover other mineral substances finely crushed and intimately admixed therewith. The carbon is then baked for hardening the core.

It is also possible to introduce inside the carbon sheath, a solid hard rod of carbon and ferrosilicon with the eventual addition of further mineral material. These substances are agglomerated by means of a binding material liable to be carbonized such as coal tar for instance. When the composition has been drawn through a press so as to form rods of suitable cross-sec-

tion, it is hardened through calcination in a reducing medium at a high temperature. The rods thus prepared are then stuck inside their sheaths.

In the following example, the final composition is defined by the proportions of mineralizing material on one hand and carbon on the other; these proportions are given out by weight.

*Example 1.*—Different anodes have received a core having the following composition:

Table I

| No.                    | I  | II | III |
|------------------------|----|----|-----|
| Ferrosilicon at 25% Si | 50 | 68 | 80  |
| Carbon                 | 50 | 32 | 20  |

Anodes the diameter of which is 7 mm. as in common use for cinematographic projections have spontaneously produced the Beck effect for normal intensities of 40–50 amperes. With the new anode in conformity with the invention, and for a same length of arc as for the anode chosen for comparison, a higher drop in voltage is observed which lies between 2 and 4 volts according to the intensity used while the luminous efficiency lies between 95–98% and 70% of that of the test anode formed with only rare earths, said efficiency decreasing with increasing current densities.

*Example 2.*—By replacing weight for weight in the Formulae I, II, III, the ferrosilicon at 25% by that containing 45% of silicon, the compositions I bis, II, bis, III bis are obtained. The resulting arcs are comparable to those of the corresponding compositions I, II, III; thus for anodes of 7 mm. the composition I bis operating under 40 amperes has provided 3% less light than the composition I but 6% more at 50 amperes. The very high contents of ferrosilicon at 45% have lesser advantages as concerns efficiency, chiefly for high current densities.

*Example 3.*—Rare earths of the ceric group under the form of commercial fluoride are associated with ferrosilicon containing 25% silicon, which leads to the following compositions:

Table II

| No.             | IV | V  | VI |
|-----------------|----|----|----|
| Ceric fluorides | 10 | 20 | 30 |
| Ferrosilicon    | 70 | 60 | 41 |
| Carbon          | 20 | 20 | 20 |

The luminous efficiency when compared with the test anode comprising only rare earths increases with the contents of the latter and reach and pass beyond those of the test anode in the case of the composition VI. In the case of anodes of 7 mm. the following results are obtained:

Table III

| Intensity | IV | V  | VI  | Test (comparison base) |
|-----------|----|----|-----|------------------------|
| 40 a      | 88 | 87 | 113 | 100                    |
| 45 a      | 67 | 80 | 98  | 100                    |
| 50 a      | 60 | 74 | 97  | 100                    |

The composition VI is therefore at least equal to the composition having rare earths as a base. But the latter containing about 60–70% of rare earths are much less economical. All the comparisons have been made with anodes of the

standard commercial type known under the trade name "Orlux 544."

*Example 4.*—By substituting weight for weight ferrosilicon at 45% for that containing 25% of silicon, one obtains the compositions IV bis, V bis, VI bis, which are respectively similar to compositions IV, V, VI. For anodes of 7 mm. diameter and under same conditions for comparisons, the following results are obtained for 40 and 50 amperes.

Table IV

| Intensity | IV bis | V bis | VI bis | Test (comparison base) |
|-----------|--------|-------|--------|------------------------|
| 40 a      | 92     | 98    | 122    | 100                    |
| 50 a      | 61     | 72    | 98     | 100                    |

The composition VI bis operating under 40 amperes produces substantially the same light as the test anode under 45 amperes.

It is possible thus with the new anodes, as desired, to save electric energy or else to benefit by an increase in luminous efficiency.

The influence of ferrosilicon at 45% on the voltage at the terminals of the arc remains of the same magnitude as that of ferrosilicon at 25%: the increase is all the greater when the proportion of rare earths contained in the core is smaller.

The advantages of the invention will appear from the following indications. It is possible to choose a composition rich in rare earths with enough ferrosilicon for increasing the brilliancy of the crater as compared to the standard anode. The composition VII containing 38% of compounds of rare earths and 41% of silicon at 45% ferrosilicon with 21% of carbon provides the results recorded in Table V. Said table shows the comparison between the usual anodes having diameters of 6, 7 and 8 mm. operating at different current intensities of 30 to 65 amperes, the light intensities being given out as percentages of that provided by the test carbons containing only rare earths of the standard grade already mentioned "Orlux 544."

Table V

| Diameter of the anode in mm. | Intensity of the current in amperes |     |     |     |     |    |    |
|------------------------------|-------------------------------------|-----|-----|-----|-----|----|----|
|                              | 30                                  | 35  | 40  | 45  | 50  | 55 | 65 |
| 6                            | 112                                 | 106 | 96  | 105 | 103 | —  | —  |
| 7                            | —                                   | —   | 119 | 105 | 103 | —  | —  |
| 8                            | —                                   | —   | —   | —   | 105 | 82 | —  |

On the contrary, if an allowable fraction of the luminous efficiency is sacrificed, it is possible to use a composition containing less rare earths which leads to a substantial economy. In particular, it is possible to use a composition VIII containing about 21% of compounds of rare earths, 53% of ferrosilicon containing 45% Si and 26% of carbon. This composition allows as a matter of fact an economy of 53 to 62% of the rare earths, taking into account all the variable interfering conditions.

It is finally possible to choose intermediary compositions, those containing the less rare earths leading to the most important economies at the expense of the luminous efficiency while those containing the most rare earths lead to a smaller but yet substantial economy with a high luminous efficiency. For the composition VII, this

economy varies between 10 and 20% according to the conditions of use.

In the economical position of to-day, the novel compositions described are of advantage as the rare earths are generally imported by sea from long distances. The use of ferrosilicons as partial or complete substitutes for the rare earths allows thus such importations to be done away with partly or totally.

In particular, if it is desired to totally eliminate the rare earths, while retaining the same luminous efficiency, it is sufficient to use ferrosilicon-containing anodes with mean current densities for instance:

1 a./mm.<sup>2</sup> for  $\phi$  6 mm. diameter  
0.9 a./mm.<sup>2</sup> for  $\phi$  7 mm. diameter  
0.8-0.85 a./mm.<sup>2</sup> for  $\phi$  8 mm. diameter  
0.75-0.8 a./mm.<sup>2</sup> for  $\phi$  9 mm. diameter  
0.65-0.70 a./mm.<sup>2</sup> for  $\phi$  13 mm. to 16 mm. diameter.

When it is desired to operate with higher current densities without reducing the luminous efficiency, it is preferable for the ferrosilicon to be used in proportions which are lower when the rate of utilization, i. e., the density of current, is higher, provided there are incorporated simultaneously rare earths. Whatever the rate of operation may be, there is always an economy made in rare earths, taking into account all the modifications which may appear for instance in the density of the core and in the rate of combustion of the coal.

The association of ferrosilicons with rare earths is also preferable when a supply of low voltage current is available as is often the case in projection halls. For this kind of application, the above referred to composition VIII is particularly available.

Generally speaking, it has been found that ferrosilicon has a remarkable stabilizing action on the arcs which considerably reduces the fluctuations in light produced by the rare earths in intense arcs.

On the other hand, it is known that the coupling of two similar anodes of the normal intense type allows the obtention of an alternating intense arc. Experience has shown that anodes with pure ferrosilicon are not suitably applicable in such a case. Anodes containing ferrosilicons with a sufficient amount of rare earths are perfectly satisfactory. For instance, the composition VIII has provided with 8 mm. carbons a luminous efficiency which is higher by 6% than that of the test anode "Orlux 542" containing rare earths, under an intensity of 80 amperes; for 85 amperes the efficiency falls underneath that of the test anode. This composition allows a clear economy of 10% in rare earths.

In addition to the principal components which are ferrosilicon and compounds of rare earths, it is possible to incorporate to the cores of the improved anodes, metals having atomic numbers comprised between 22 and 29 or alloys of such metals with one another or with silicon. The results are similar but the corresponding anodes are more expensive and generally speaking of minor advantages for general utilization, so that they should be reserved for special applications.

Of course the present invention is by no means limited to the form of execution and numeric values given out by way of examples. The different details of execution and application may vary as desired without widening the scope of the invention.

What I claim is:

1. An anode for intensive electric arcs adapted to produce spontaneously the Beck effect, comprising a sheath of carbon and a core constituted by a base of commercially pure carbon admixed with an inoxidable ferrous alloy.
2. An anode for intensive electric arcs adapted to produce spontaneously the Beck effect, comprising a sheath of carbon and a core constituted by a base of commercially pure carbon admixed with an inoxidable ferrous alloy, containing at least one metal having an atomic number comprised between 22 and 29 inclusively.
3. An anode for intensive electric arcs adapted to produce spontaneously the Beck effect, comprising a sheath of carbon and a core constituted by a base of commercially pure carbon admixed with ferrosilicon rich in silicon.
4. An anode for intensive electric arcs adapted to produce spontaneously the Beck effect, comprising a sheath of carbon and a core constituted by a base of commercially pure carbon admixed with an inoxidable ferrous alloy and rare earths.
5. An anode for intensive electric arcs adapted to produce spontaneously the Beck effect, comprising a sheath of carbon and a core constituted by a base of commercially pure carbon admixed with a ferrosilicon containing between about 25 and 45% of silicon and compounds of rare earths.
6. An anode for intensive electric arcs adapted to produce spontaneously the Beck effect, comprising a sheath of carbon and a core constituted by a base of commercially pure carbon admixed with a ferrosilicon containing between about 25 and 45% of silicon and a metal the atomic number of which is comprised between 22 and 29.
7. An anode for intensive electric arcs adapted to produce spontaneously the Beck effect, comprising a sheath of carbon and a core constituted by a base of commercially pure carbon admixed with a ferrosilicon containing between about 25 and 45% of silicon, compounds of rare earths and a metal the atomic number of which is comprised between 22 and 29 inclusively.
8. An anode for intensive electric arcs adapted to produce spontaneously the Beck effect, comprising a sheath of carbon and a core constituted by a base of commercially pure carbon admixed with ferrosilicon and alloys of a metal having an atomic number comprised between 22 and 29 inclusively.
9. An anode for intensive electric arcs adapted to produce spontaneously the Beck effect, comprising a sheath of carbon and a core constituted by a base of commercially pure carbon admixed with ferrosilicon and alloys of a metal having an atomic number comprised between 22 and 29 inclusively and silicon.
10. An anode for intensive electric arcs adapted to produce spontaneously the Beck effect, comprising a sheath of carbon and a core constituted by a base of commercially pure carbon admixed with ferrosilicon, alloys of a metal having an atomic number comprised between 22 and 29 inclusively and rare earths.
11. A composition for the core of anodes adapted for use in intensive arcs producing the Beck effect containing about 50 to 80% of ferrosilicon with silicon contents between 25 and 45% and 50 to 20% of commercially pure carbon.
12. A composition for the core of anodes adapted for use in intensive arcs producing the Beck effect containing between about 10 to 40% of compounds of rare earths, between about 70 and 40% of ferrosilicon having contents com-

prised substantially between 25 and 45% and about 20% of carbon.

13. An anode for intensive electric arcs adapted to produce spontaneously the Beck effect, comprising a sheath of carbon and a core constituted by a base of commercially pure carbon admixed with a ferrosilicon containing between about 25 and 45% of silicon.

14. An anode for intensive electric arcs adapted to produce spontaneously the Beck effect, comprising a sheath of carbon and a core containing about 38% of compounds of ceric earth, about 41% of ferrosilicon containing about 45% of silicon, and about 21% of carbon.

15. An anode for intensive electric arcs adapted to produce spontaneously the Beck effect, comprising a sheath of carbon and a core containing about 21% of rare earths, about 53% of ferrosili-

con containing 45% of silicon and about 26% of carbon.

JEAN FRANÇOIS PARISOT.

#### REFERENCES CITED

The following references are of record in the file of this patent:

#### UNITED STATES PATENTS

| Number    | Name    | Date          |
|-----------|---------|---------------|
| 955,273   | Ladoff  | Apr. 19, 1910 |
| 2,140,881 | Parisot | Dec. 20, 1938 |

#### FOREIGN PATENTS

| Number  | Country       | Date          |
|---------|---------------|---------------|
| 456,040 | Great Britain | Nov. 2, 1936  |
| 475,252 | Great Britain | Nov. 16, 1937 |